

May 1, 1923.

1,453,699

O. BROPHY

## METHOD FOR SEPARATING MAGNETIC MATERIALS

Filed Sept. 28, 1921

FIG. 1.



FIG. 2.



Inventor

*Oscar Brophy*

३५१

F. DeWitt Goodwin

Attorney

Patented May 1, 1923.

1,453,699

# UNITED STATES PATENT OFFICE.

OSCAR BROPHY, OF PHILADELPHIA, PENNSYLVANIA.

METHOD FOR SEPARATING MAGNETIC MATERIALS.

Application filed September 28, 1921. Serial No. 503,883.

To all whom it may concern:

Be it known that I, OSCAR BROPHY, a citizen of the United States, residing at Philadelphia, in the county of Philadelphia and 5 State of Pennsylvania, have invented certain new and useful Improvements in the Method for Separating Magnetic Materials, of which the following is a specification.

My invention relates to the separation of 10 material by means of a magnetic separator, and my invention particularly relates to the method of separating magnetic metals having different critical temperatures, by heating the metals sufficiently to render one of 15 the metals temporarily non-magnetic and passing the metals through the separator in this state, whereby the separator will cause the magnetic and non-magnetic metals to be deflected into different channels in the usual 20 manner.

The object of my invention is to provide a method for separating metals, such as 25 Monel metal from iron, whereby the loose particles of different materials in the form of borings, filings, lathe turnings and the like, may be readily separated; and a further object of my invention is to provide an apparatus for carrying out the above 30 mentioned method of separating materials, comprising a heating device for heating the metals in which exhaust steam may be utilized for this purpose at a low cost of operating the apparatus.

In carrying out my invention, sufficient 35 heat may be derived from steam pipes, or a steam heated jacket, to render the Monel metal non-magnetic, as this metal ceases to be magnetic at two hundred and five degrees F., approximately.

Referring to the accompanying drawing, Fig. 1, is a vertical sectional view of a magnetic separator embodying a heating device, and Fig. 2 is a plan view of Fig. 1.

In the accompanying drawings, in which 45 like reference characters refer to like parts, 1 represents one form of a magnetic separator, now in general use, which comprises a frame 2 on which is mounted pulleys 3 and 4, rotated in any suitable manner and around 50 the pulleys extends an endless belt 5. The pulley 4 is a magnetic pulley and contains any suitable form of magnets 6, adapted to attract magnetic material, carried by the belt 5, around said pulley 4, a sufficient distance to cause it to be drawn out of the vertical line or path through which the non-

magnetic material will fall from the belt 5 and thus separate the two materials and deposit them in separate compartments 7 and 8.

A hopper 10 is positioned above the belt 5 for receiving the mingled material and distributing the same upon the belt 5.

In carrying out my invention, I construct the hopper 10, with a jacket 12, which forms a chamber 13 around the hopper 10. A steam supply pipe 14 and an outlet pipe 15 are connected with the chamber 13 of the hopper, whereby steam may be circulated through the chamber 13 for heating the hopper 10, and the material as it passes through the hopper.

The hopper is positioned close to the magnetic pulley 4 so that the material will pass over the pulley before it cools.

Monel metal, consisting essentially of copper and nickel, is now extensively used in the various manufactures, and it is desirable to save the large amount of waste of this material in the form of borings and turnings, which have heretofore been discarded, due to the presence of the iron and steel mingled therewith, which rendered the Monel metal, containing such scrap metal, uneven in texture and difficult to machine, due to the hard spots therein caused by the high percentage of iron.

By my novel method of separating metals; Monel metal, and metals of similar character, may be reclaimed from scrap containing iron and steel by heating the same sufficiently to render one of the metals temporarily non-magnetic and passing the mingled substances through a magnetic separator while heated.

I do not confine myself to heating by exhaust steam, but may use any of the well known methods for heating.

Having thus described my invention, I claim and desire to secure by Letters Patent:

1. The method of separating two magnetic substances by means of a magnetic separator, comprising the heating of the substances to a sufficient temperature to render one of said substances non-magnetic without change of composition and passing the substances through the separator while heated.

2. The method of separating two magnetic substances by means of a magnetic separator, comprising the heating of the substances to a sufficient temperature to

render one of said substances temporarily non-magnetic without change of composition, and passing the substances through the separator while heated.

3. The method of separating magnetic metals, comprising the heating of the mingled metals to a temperature which will render one of the metals non-magnetic without changing the composition and passing 10 the same through a magnetic separator while heated.

4. The method of separating Monel metal from other magnetic metals, comprising the heating of the mingled metals to a temperature 15 which will render the Monel metal non-magnetic without changing its composition, and passing the same through a magnetic separator while heated.

5. The method of separating a substance 20 composed of essentially copper and nickel from another metal such as iron, comprising the heating of the mingled substances without changing the composition to a temper-

ature which will temporarily render the first named substance non-magnetic and passing 25 the mingled substances through a magnetic separator whereby the iron will be acted upon by the magnet of the separator, and the first named substance will pass through the separator without being affected by the 30 said magnet.

6. The method of separating two substances having different magnetic critical temperatures, comprising heating the mingled substances without changing the composition to 35 a temperature which will render one of the substances non-magnetic without affecting the magnetic state of the other substance, and passing the mingled substances through a magnetic separator for separating the magnetic substance from the substance rendered 40 temporarily non-magnetic by the increase of temperature.

In testimony whereof I affix my signature.

OSCAR BROPHY.